# EUROPEAN PATENT SPECIFICATION

(11) **EP 0 529 009 B1**
(45) Date of publication and mention of the grant of the patent: **06.04.1994**
(21) Application number: 91920968.4
(22) Date of filing: 01.05.1991
(51) Int. Cl.: G03C 7/30, G03C 5/395

(54) **IMPROVEMENTS RELATING TO A PHOTOGRAPHIC PROCESS**
VERBESSERUNGEN IN BEZUG AUF EIN PHOTOGRAPHISCHES VERFAHREN
TRAITEMENT PHOTOGRAPHIQUE AMELIORE

(30) Priority: 30.04.1990 GB 9009678
(43) Date of publication of application: 03.03.1993
(73) Proprietor: KODAK LIMITED, Hemel Hempstead Hertfordshire HP1 1JY (GB); EASTMAN KODAK COMPANY, Rochester, New York 14650-2201 (US)
(72) Inventor: FYSON, John, Richard "Tortworth", London E8 7AS (GB)
(74) Representative: Daley, Michael John
(86) International application number: EP9100845
(87) International publication number: WO9117479

(56) References cited:
- EP-A- 0 128 720
- GB-A- 1 514 517
- US-A- 4 147 546
- US-A- 4 529 687
- Patent Abstracts of Japan, Vol. 1, no. 44() 27 April 1977,& JP-A-51 140732
- Patent Abstracts of Japan, vol. 2, no. 42() 20 March 1978, & JP-A-53 008135
- Derwent Japanese Patents Report, vol. 80, no. 3, 15 February 1980, Derwent Publications, Section Chemical, London, GB, & JP-B-80 001571
- SMPTE Journal, vol. 94, no. 6, June 1985, US, pp. 648-653; J.L. Burger et al: "Recovery of Kodak color developing agent CD-2 from process ECP-2A colordeveloper and stop bath"
- Journal of Imaging Technology, vol. 10, no. 6, December 1984, Springfield, US, pp. 217-221; K.L. Wahl et al: "RSMP-A modular system for recycling and treatment of photographic effluents"

## Description

The invention relates to a photographic process of the kind in which a silver halide material carried on a photographic carrier material is treated with a developer to develop an image and is then passed to an amplification bath. Subsequent to the amplification bath, the material is passed to a fixing and washing stage.

During a process of this kind the amplification bath itself has developer carried over into it which is transported on the material being processed and the presence of this developer builds up and shortens the life of the amplifier bath. In order to keep the bath up to the right strength it has to be replenished periodically to compensate for this build-up of developer.

If developer is retained on the material and is not removed completely by the end of the photographic process there is the risk that the final print material obtained will be liable to subsequent staining as the retained developer in the gelatine or its carrier will, under certain conditions, such as exposure to heat and light, cause further action by the developer which reacts with the constituents of the material to give an effect known as staining or a deeper intensity of certain colours. This is clearly not desirable since any photographic print is needed to remain stable over a long period and over a reasonable range of temperature and light conditions.

It is an object of the present invention to provide an improvement in a photographic process of the above kind which uses an amplification bath in which the problems associated with the build-up of developing agent are substantially reduced.

In GB-A-1,514,517 there is described a photographic development process wherein a photographic material is treated with a developer agent and subsequently passed to an in-line amplification bath comprising hydrogen peroxide.

The present invention is characterised in that the amplification bath is treated with an ion exchange resin to reduce the amount of available developer agent retained in the bath.

The absorbing agent is preferably an ionic exchange resin, which may be either cationic, anionic or neutral. In certain circumstances, a mixture of anionic and cationic resins may operate successfully.

It has been known to use these absorbing agents for the treatment of waste solutions and to remove the colour developing agent from these waste solutions.

For example, in U.S. Patent Specification No. 4606827 the use of a cation exchange resin is disclosed with a solution which has a pH value not exceeding 8.0 for selective operation of a phenylenediamine colour developing agent to prevent the pollution of discharged waters into public sewers.

In British Patent Specification No. 2054182A the use of an ion exchange resin is disclosed to remove the degradation products of a developer in a fixer after the fixer has been subject to electrolysis to remove the dissolved silver in it.

None of the prior art shows the use of ion exchange resins in the tail-end of a photographic process which includes an amplification bath. The following example illustrates the effect of different absorbing materials when used to remove the colour-developing agent when used in an amplification bath:

### EXAMPLE

A simulated seasoned amplification bath was made by adding 100mls. of an 'RX' developer to 500mls of an amplifier suitable for use with low silver materials. The formulae are as follows :

### Developer :

- potassium carbonate: 30.0g
- sodium sulphite: 2.0g
- disodium EDTA: 0.1g
- CD3: 8.0g
- water to: 1.0 litre

pH adjusted to 10.3 with potassium hydroxide solution

### Amplifier :

- hydrogen peroxide (100 vol): 30mls
- water to: 1.0 litre

50mls samples of the amplifier/developer mixture were stirred with 5g of different resins for 10 minutes. The residual CD3 in the fixer mixture was determined by HPLC.

The results are tabulated below:

It will be seen from the above example that the absorbing agents all had an effect to a greater or lesser degree in reducing the amount of agent in the amplification bath. Clearly a selection of suitable agent has to be made depending on the nature of the developer in each bath. For the 'RX'developer selected for this example there are five absorbing ion exchange resins which are wholly successful in removing all the developing agent.

This enables the amplification bath to have a much longer life than would otherwise be the case and reduces the amount of replenishment which is necessary for it, thus increasing the economics of the process. Furthermore, there will be no staining caused by a build-up of any developing agent in the material.

## Claims

1. A photographic development process wherein a photographic material is treated with a developer agent and subsequently passed to an in-line amplification bath comprising hydrogen peroxide, characterized in that the amplification bath is treated with an ion exchange resin to reduce the amount of available developer agent retained in the bath.

2. A process as claimed in claim 1 characterized in that the ion exchange resin is cationic.

3. A process as claimed in claim 1 characterized in that the ion exchange resin is anionic.

4. A process as claimed in claim 1 characterized in that the ion exchange resin is neutral.

5. A process as claimed in claim 1 characterized in that the ion exchange resin is a mixture of cationic and anionic resins.

## Patentansprüche

1. Photographisches Entwicklungsverfahren, bei dem ein Photomaterial mit einem Entwicklungsmittel behandelt und anschließend zu einem Wasserstoffperoxid enthaltenden In-line-Verstärkungsbad geleitet wird,
dadurch **gekennzeichnet,**
daß das Verstärkungsbad mit einem Ionenaustauschharz behandelt wird zum Verringern der Menge an im Verstärkungsbad zurückgehaltenem verfügbarem Entwicklungsmittel.

2. Verfahren nach Anspruch 1, dadurch gekennzeichnet, daß das Ionenaustauschharz kationisch ist.

3. Verfahren nach Anspruch 1, dadurch gekennzeichnet, daß das Ionenaustauschharz anionisch ist.

4. Verfahren nach Anspruch 1, dadurch gekennzeichnet, daß das Ionenaustauschharz neutral ist.

5. Verfahren nach Anspruch 1, dadurch gekennzeichnet, daß das Ionenaustauschharz ein Gemisch aus kationischen und anionischen Harzen ist.

## Revendications

1. Procédé de développement photographique dans lequel le matériau photographique est traité avec un agent révélateur puis est ensuite passé dans un bain d'amplification comprenant du peroxyde d'hydrogène, caractérisé en ce que le bain d'amplification est traité avec une résine échangeuse d'ions pour réduire la quantité d'agent révélateur disponible retenue dans le bain.

2. Procédé selon la revendication 1, caractérisé en ce que la résine échangeuse d'ions est cationique.

3. Procédé selon la revendication 1, caractérisé en ce que la résine échangeuse d'ions est anionique.

4. Procédé selon la revendication 1, caractérisé en ce que la résine échangeuse d'ions est neutre.

5. Procédé selon la revendication 1, caractérisé en ce que la résine échangeuse d'ions est un mélange de résines cationique et anionique.
